# EUROPEAN PATENT APPLICATION

(11) **EP 2 199 376 A1**
(43) Date of publication of application: **23.06.2010**
(21) Application number: 07816782.2
(22) Date of filing: 08.11.2007
(51) Int. Cl.: C10L 1/20, C10L 1/26, C10L 1/224, C10L 1/04

(54) **AN ENVIRONMENTAL FRIENDLY LIGHT HYDROCARBON FUEL FOR VEHICLES**

(30) Priority: 10.09.2007 CN 200710045753
(71) Applicant: Shanghai Chinamax New Energy CO., LTD., No.6726 Tingwei Road Jinshan District Shanghai 201506 (CN)
(72) Inventor: LEE, Maosheng, Shanghai 201506 (CN); WU, Yenchih, Shanghai 201506 (CN); ZHAO, Jianming, Shanghai 201506 (CN); LI, Chienchih, Shanghai 201506 (CN)
(74) Representative: Gervasi, Gemma
(86) International application number: PCT/CN2007/003170
(87) International publication number: WO 2009/033331

(57) **Abstract**

The present invention discloses an environmental-friendly vehicle light hydrocarbon fuel, with contents of its components as below according to part by weight: (1) Light hydrocarbon: 100 parts by weight; (2) aromatic hydrocarbon: 4∼60 parts by weight; (3) lead free antiknock: 0∼20 parts by weight; (4) cation fluorocarbon surfactant: 0∼0.2 parts by weight; and (5) surface active increased superscript agent: 0.001∼2 parts by weight. The product of the present invention can increase auto-ignition temperature of the fuel, improve distillation range distribution of the fuel, increase burning velocity of the fuel, enhance power and reduce abrasion of an engine, avoid the formation of piston carbon, and lower consumption of the fuel, with a calorific value ≥ 42000 KJ/kg, being a novel substitute vehicle fuel that is energy saving, environmental-friendly, and cost effective.

## Description

### FIELD OF THE INVENTION

The present invention relates to an environmental-friendly vehicle light hydrocarbon fuel, more particularly, relates to the environmental friendly vehicle light hydrocarbon fuel with the main components being pentane and heavier hydrocarbons that is extracted from condensate of a petrochemical plant or of the natural gas,.

### BACKGROUND OF THE INVENTION

Since August 1, 2006 in China, the two cities, Beijing and Shanghai, have taken the lead in executing the national standard of vehicle pollutant emission (the National III Standard). A vehicle consuming gasoline is not easy to reach the National III Standard because a high boiling component, with a wide distillation range, is inclined to produce CO and HC during combustion. Light hydrocarbon has little emission of CO and HC pollutants because of its low distillation range, low boiling point as well as complete combustion, and thus the limit value of emission (the National III Standard) can be reached.

### SUMMARY OF THE INVENTION

The technical problem to be solved by the present invention is to disclose an environmental-friendly vehicle light hydrocarbon fuel, so as to overcome the above-mentioned shortcomings and environmental pollution problems in the prior art, and satisfy requirements of related aspects.

The technical problem to be solved by the present invention can be overcomed through the following technical solution:

An environmental-friendly vehicle light hydrocarbon fuel is provided, which is **characterized in that** contents of the components are as below according to part by weight:
(1) Light hydrocarbon: 100 parts by weight;
(2) Aromatic hydrocarbon: 4∼60 parts by weight;
(3) Lead free antiknock: 0∼20 parts by weight;
(4) Cation fluorocarbon surfactant: 0∼0.2 parts by weight; and
(5) Surface active increased superscript agent: 0.001∼2 parts by weight.

The light hydrocarbon according to the present invention, with the main components being pentane and heavier hydrocarbons, is a fraction extracted from condensate of a petrochemical plant or of the natural gas, with the main components being pentane and heavier hydrocarbons and the RON being 50∼80.

The aromatic hydrocarbon according to the present invention includes toluene, xylene, or hybrid aromatic hydrocarbons for producing toluene.

The lead free antiknock according to the present invention includes methyl tert-butyl ether (MTBE), tert-amyl methyl ether (TAME), tert-butyl alcohol, isobutanol, and anhydrous methanol or anhydrous ethanol. 1.

The cation fluorocarbon surfactant according to the present invention, being fluorinated alkyl amine salt or quaternary ammonium salt cation fluorocarbon surfactant, is selected from the substances with a formula (1), (2) or (3) or mixture thereof. The content of the cation fluorocarbon surfactant, is generally 0∼0.2 parts by weight, preferably 0∼0.1 parts by weight based on 100 parts by weight of the light hydrocarbon.
(1) Quaternary ammonium salt-type cation fluorocarbon surfactant containing fluorinated alkyl amine:

   (CF₃)₂CF(CF₂)₆CH₂CH(OH)CH₂N⁺(CH₃)₃I⁻
(2) Perfluorinated alkyl amide quaternary ammonium salt-type cation fluorocarbon surfactant:

   C₇F₁₅CONH(CH₂)₃N⁺(CH₃)₃I⁻
(3) Fluorinated alkyl amine salt type cation fluorocarbon surfactant:

   [F(CF₂)₈CH(OH)CH₂]₂NCH₂CH₂NH₂·1/2H₂SO₄

The surface active increased superscript agent according to the present invention is obtained by mixing one of components ① ∼ ⑥ and a component ⑦, wherein the content ratio of one of the components ① ∼ ⑥ to the component ⑦ is 100:60∼80 parts by weight. The content of the surface active increased superscript agent is generally 0.001∼2 parts by weight, preferably 0.01∼0.2 parts by weight, based on 100 parts by weight of the light hydrocarbon.
① C₈F₁₇SO₂N(CH₃)CH₂OP(O)(OH)₂
② C₈F₁₇SO₂N(CH₃)CH₂OP(O)(ONa)₂
③ C₈F₁₇SO₂N(CH₃)CH₂CH₂OP(O)(OH)₂
④ C₈F₁₇SO₂N(CH₃)CH₂CH₂OP(O)(ONa )₂
⑤ C₈F₁₇SO₂N(C₂H₅)CH₂CH₂OP(O)(OH)₂
⑥ C₈F₁₇SO₂N(C₂H₅)CH₂CH₂OP(O)(ONa)₂
⑦ C₁₇H₃₅CONH(CH₂)₂NHCOC₁₇H₃₅

The method of preparing the environmentally safe vehicle light hydrocarbon fuel according to the present invention is a kind of physical mixing method, which is realized by mixing various raw materials.

With the surface active increased superscript agent, the environmental friendly light hydrocarbon fuel of the present invention, whose Research Octane Number (RON) is not lower than 93, is suitable for a vehicle engine with various compression ratio, and becomes an environmental friendly vehicle light hydrocarbon fuel.

The environmental friendly vehicle light hydrocarbon fuel containing the surface active increased superscript agent can increase auto-ignition temperature of the fuel, improve distillation range distribution of the fuel, increase burning rate of the fuel, enhance power and reduce abrasion of an engine, avoid the formation of piston carbon, and lower consumption of the fuel, with a calorific value ≥ 42000 KJ/kg, being a novel substitute vehicle fuel that is energy saving, environmental friendly, and cost effective.
the contents of the exhaust pollutants of the environmental friendly vehicle light hydrocarbon fuel according to the present invention-, are much lower than the GB18352.3-2005 Standard, based on test of contents of the exhaust pollutants CO, HC, and NOₓ.

| | Unit | Experimental result | National standard requirement of P.R. China |
|---|---|---|---|
| CO | g/km | 1.209 | ≦ 2.3 |
| HC | g/km | 0.075 | ≦ 0.20 |
| NOₓ | g/km | 0.046 | ≦ 0.15 |

The surface active increased superscript agent can be substituted by the following components ⑧, ⑨, ⑩ or mixture thereof in the environmental friendly vehicle light hydrocarbon fuel according to the present invention, so as to reduce the cost:
⑧ C₈F₁₇SO₂NHCH₂CH₃
⑨ C₈F₁₇SO₃K
⑩ C₈F₁₇SO₃N(C₂H₅)₄

### DETAILED DESCRIPTION OF THE EMBODIMENTS

### Example 1

(1) Light hydrocarbon (the RON is 70): 100 parts by weight;
(2) Toluene: 30 parts by weight;
(3) Cation fluorocarbon surfactant: 0.006 parts by weight; and
(4) Surface active increased superscript agent: 0.05 parts by weight.

In example 1, the light hydrocarbon is a fraction extracted from condensate of a petrochemical plant or of the natural gas, with the main components being pentane and heavier hydrocarbons.

In example 1, the cation fluorocarbon surfactant is quaternary ammonium salt-type cation fluorocarbon surfactant containing the fluorinated alkyl amine:

(CF₃)₂CF(CF₂)₆CH₂CH(OH)CH₂N⁺(CH₃)₃I⁻

In example 1, the surface active increased superscript agent is as below:

③ C₈F₁₇SO₂N(CH₃)CH₂CH₂OP(O)(OH)₂

⑦ C₁₇H₃₅CONH(CH₂)₂NHCOC₁₇H₃₅

In example 1, the weight ratio of the surface active increased superscript agent ③ to the component ⑦ is 10:6.

The product is then obtained by mixing the components (1), (2), (3) and (4), with the Research Octane Number (RON) being 93.

### Example 2

(1) Light hydrocarbon (the RON is 70): 100 parts by weight;
(2) Xylene: 20 parts by weight;
(3) MTBE: 10 parts by weight;
(4) Cation fluorocarbon surfactant: 0.006 parts by weight; and
(5) Surface active increased superscript agent: 0.09 parts by weight.

In example 2, the light hydrocarbon is a fraction extracted from condensate of a petrochemical plant or of the natural gas, with the main components being pentane and heavier hydrocarbons.

In example 2, the cation fluorocarbon surfactant is as below:
Perfluorinated alkyl amide quaternary ammonium salt-type cation fluorocarbon surfactant:

   C₇F₁₅CONH(CH₂)₃N⁺(CH₃)₃I⁻

In example 2, the surface active increased superscript agent is as below:

① C₈F₁₇SO₂N(CH₃)CH₂OP(O)(OH)₂

⑦ C₁₇H₃₅CONH(CH₂)₂NHCOC₁₇H₃₅

In example 2, the weight ratio of the surface active increased superscript agent ① to the component ⑦ is 10:6.

The product is then obtained by mixing the components (1), (2), (3), (4) and (5) in example 2, with the RON being 93.

The exhaust pollutants of the product of the present embodiment, CO, HC and NOₓ, are tested by the test method of GB18352.3-2005, with the test results as below:

| | Unit | Experimental result | National standard requirement of P.R. China |
|---|---|---|---|
| CO | g/km | 1.209 | ≦ 2.3 |
| HC | g/km | 0.075 | ≦ 0.20 |
| NOₓ | g/km | 0.046 | ≦ 0.15 |

### Example 3

(1) Light hydrocarbon (the RON is 70): 100 parts by weight;
(2) Toluene: 30 parts by weight; and
(3) Surface active increased superscript agent: 0.1 parts by weight.

In example 3, the light hydrocarbon is a fraction extracted from condensate of a petrochemical plant or of the natural gas, with the main components being pentane and heavier hydrocarbons.

In example 3, the surface active increased superscript agent is as below:

③ C₈F₁₇SO₂N(CH₃)CH₂CH₂OP(O)(OH)₂

⑦ C₁₇H₃₅CONH(CH₂)₂NHCOC₁₇H₃₅

In example 3, the weight ratio of the surface active increased superscript agent ③ to the component ⑦ is 10:6.

The product is then obtained by mixing the components (1), (2) and (3), with the Research Octane Number (RON) being 93.

It should be explained that, what mentioned above is only the preferred embodiment of the present invention; any change that is made according to the concept of the present invention and its functional action produced is not yet out of the spirit of the specification, and should be within the scope of the present invention.

## Claims

1. An environmental friendly vehicle light hydrocarbon fuel, **characterized in that** contents of its components are as below according to part by weight:
(1) Light hydrocarbon: 100 parts by weight;
(2) Aromatic hydrocarbon: 4∼60 parts by weight;
(3) Lead free antiknock: 0∼20 parts by weight;
(4) Cation fluorocarbon surfactant: 0 ∼ 0.2 parts by weight; and
(5) Surface active increased superscript agent: 0.001∼2 parts by weight.

2. The environmental friendly vehicle light hydrocarbon fuel according to claim 1, **characterized in that** the light hydrocarbon is a fraction extracted from condensate of a petrochemical plant or of the natural gas, with the main components being pentane and heavier hydrocarbons.

3. The environmental friendly vehicle light hydrocarbon fuel according to claim 1, **characterized in that** the aromatic hydrocarbon includes toluene, xylene, or hybrid aromatic hydrocarbons for producing toluene.

4. The environmental friendly vehicle light hydrocarbon fuel according to claim 1, **characterized in that** the lead free antiknock includes methyl tert-butyl ether, tert-amyl methyl ether, tert-butyl alcohol, isobutanol, and anhydrous methanol or anhydrous ethanol.

5. The environmental friendly vehicle light hydrocarbon fuel according to claim 1, **characterized in that** the cation fluorocarbon surfactant, being fluorinated alkyl amine salt or quaternary ammonium salt type cation fluorocarbon surfactant, is selected from substances with a formula (1), (2) or (3) or mixture thereof:
(1) Quaternary ammonium salt type cation fluorocarbon surfactant containing fluorinated alkyl amine:
(CF₃)₂CF(CF₂)₆CH₂CH(OH)CH₂N⁺(CH₃)₃I⁻
(2) Perfluorinated alkyl amide quaternary ammonium salt type cation fluorocarbon surfactant:
C₇F₁₅CONH(CH₂)₃N⁺(CH₃)₃I⁻
(3) Fluorinated alkyl amine salt type cation fluorocarbon surfactant:
[F(CF₂)₈CH(OH)CH₂]₂NCH₂CH₂NH₂·1/2H₂SO₄

6. The environmental friendly vehicle light hydrocarbon fuel according to claim 1, **characterized in that** the surface active increased superscript agent is obtained by mixing one of components ① ∼ ⑥ and a component ⑦:
① C₈F₁₇SO₂N(CH₃)CH₂OP(O)(OH)₂
② C₈F₁₇SO₂N(CH₃)CH₂OP(O)(ONa)₂
③ C₈F₁₇SO₂N(CH₃)CH₂CH₂OP(O)(OH)₂
④ C₈F₁₇SO₂N(CH₃)CH₂CH₂OP(O)(ONa)₂
⑤ C₈F₁₇SO₂N(C₂H₅)CH₂CH₂OP(O)(OH)₂
⑥ C₈F₁₇SO₂N(C₂H₅)CH₂CH₂OP(O)(ONa)₂
⑦ C₁₇H₃₅CONH(CH₂)₂NHCOC₁₇H₃₅

7. The environmental friendly vehicle light hydrocarbon fuel according to claim 6, **characterized in that** the surface active increased superscript agent is obtained by mixing 100 parts by weight one of the components ① ∼ ⑥ and 60-80 parts by weight the component ⑦ according to claim 6.

8. The environmental friendly vehicle light hydrocarbon fuel according to claim 1, **characterized in that** the content of the cation fluorocarbon surfactant is preferably 0∼0.1 parts by weight based on 100 parts by weight of the light hydrocarbon.

9. The environmental friendly vehicle light hydrocarbon fuel according to claim 1, **characterized in that** the content of the surface active increased superscript agent is preferably 0.01∼0.2 parts by weight based on 100 parts by weight of the light hydrocarbon.

10. The environmental friendly vehicle light hydrocarbon fuel according to claim 1, **characterized in that** one of the following components or the mixture thereof may also be added if necessary:
⑧ C₈F₁₇SO₂NHCH₂CH₃
⑨ C₈F₁₇SO₃K
⑩ C₈F₁₇SO₃N(C₂H₅)₄
